

1

2,925,317

**SHRINKPROOFING OF PROTEIN FIBERS WITH POLYALKYLENEIMINES**

Joseph E. Moore, Pinole, and Clay E. Pardo, Jr., Albany, Calif., assignors to the United States of America as represented by the Secretary of Agriculture

No Drawing. Application September 18, 1956  
Serial No. 610,690

4 Claims. (Cl. 8—127.6)

(Granted under Title 35, U.S. Code (1952), sec. 266)

A non-exclusive, irrevocable, royalty-free license in the invention herein described, throughout the world for all purposes of the United States Government, with the power to grant sublicenses for such purposes, is hereby granted to the Government of the United States of America.

This invention relates to processes for shrinkproofing and felt-proofing proteinaceous fibers, especially wool. In particular, the invention is concerned with procedures wherein the fiber is treated with a preformed polyalkyleneimine and then cured with the application of heat whereby to produce a fiber which exhibits a marked resistance to shrinkage as compared with the original fiber. Further objects and advantages of the invention will be obvious from the description herein.

It is well known that laundering causes severe shrinkage to woolen textiles. This technical disadvantage seriously restricts the applications of wool in the textile industry and much research has been undertaken to modify the natural fiber to improve its shrinkage properties. In general, known methods of treating wool to improve its shrinkage characteristics have the disadvantage that the hand of the fabric is impaired. This is particularly true where resins are applied to the textile.

It has now been found that if wool is treated with a preformed polyalkyleneimine, the shrinkage characteristics of the fiber are drastically improved. It has further been found that maximum shrinkproofing effect is attained when the preformed polyalkyleneimine is applied to the fiber as a solution having a controlled pH and when the imine-treated wool is subjected to a heat curing operation. Under these circumstances, the treated wool is almost completely shrinkproof under usual laundering procedures. The reason for the effectiveness of the process of this invention cannot be explained on a scientific basis. However, it is believed that the polyalkylene imine actually reacts with the wool, forming part of the protein molecule. This view is substantiated by the fact that the original imine applied to the wool is water-soluble, whereas after treatment, the imine cannot be removed from the wool by washing with hot water or by laundering. Additional advantages of the process of the invention are that the treated wool is not impaired for its intended purposes. Thus its tensile strength and hand are not adversely affected.

In applying the process of this invention, the wool is impregnated with a solution of the preformed polyalkyleneimine. The treatment is advantageously performed by immersing the wool in an excess of the solution or by applying the solution by spraying, brushing or other conventional application techniques. To assist in wetting the wool with the solution, it may be run through padding rolls or the like.

Although polyethylene imine is the preferred shrinkproofing agent of this invention, one can use any other polyalkylene imine. Typical examples are the polymers of: propylene imine; 1,2-butylene imine; 2,3-butylene

2

imine; 2,2-dimethyl-ethylene imine; 2,2,3-trimethyl-ethylene imine; 2,2-dimethyl-3-propyl-ethylene imine; cyclohexyl-ethylene imine; phenyl ethylenimine, etc. These compounds, as well known in the art, can be prepared, for example, by polymerizing the alkylene imine in the presence of a catalyst such as sodium bisulphite, hydrochloric acid, sulphuric acid, acetic acid, hydrogen peroxide, and so forth. Generally, it is preferred to use the polyalkylene imines which are at least partially soluble in water.

10 The solution applied to the protein fibers in accordance with this invention contains as its principal ingredient the preformed polyalkylene imine. The concentration of this agent in the solution is not critical and may be, for example, as low as 0.1% or as high as 10%. Usually water is used as the sole solvent for the imine. However, the solution may contain both water and a water-soluble organic solvent such as methyl alcohol, ethyl alcohol, propyl alcohol, isopropyl alcohol, any of the isomeric butyl alcohols, acetone, etc. The use of a mixed solvent of water and alcohol or ketone is particularly useful where the particular imine chosen is not completely water-soluble.

20 In order to achieve a maximum shrinkproofing effect, it is necessary to control the pH of the polyalkylene imine solution which is applied to the protein fiber. Acid conditions are not suitable as they prevent production of a shrink-resistant product. To achieve best results, the treating solution should be preferably alkaline, that is, the pH should be in the range about from 9 to preferably about 11. The polyalkylene imines exhibit an alkaline reaction when dissolved in water and in most cases it is unnecessary to add any agent to control the pH. Where, however, it is desired or necessary to adjust the pH to the above-cited range, one may add to the treatment solution an acid or alkaline substance as needed. To decrease the pH, one may add agents such as sulphuric acid, hydrochloric acid, phosphoric acid, sodium bisulphite, monosodium phosphate, etc. To increase the pH one may add such agents as sodium carbonate, trisodium phosphate, borax, potassium carbonate, tetrasodium pyrophosphate, and so forth.

30 After the wool has been impregnated with the imine solution, it is subjected to a heat curing operation. This simply involves subjecting the textile material to a temperature from about 75 to about 150° C. to promote reaction between the imine and the wool whereby the imine becomes bonded to the protein molecule and can no longer be removed by washing. The time of cure will vary depending on the temperature selected, the chemical nature of the fiber being treated, the degree of shrinkproofing desired, and so on. In general, a cure time of about 15 min. to about 2 hours may be used. A preferred curing operation involves heating for about 30 minutes to one hour at 120° C.

40 After the textile material has been cured it may be washed with water or laundered to remove excess imine which is not actually bonded to the protein molecules. The textile material is then dried in the usual manner and is ready for use.

50 The proportion of polyalkylene imine bonded to the protein fiber may be varied widely by varying the concentration of polyalkyleneimine in the treatment solution taken up by the fibrous material. Usually these conditions are so chosen that the fiber takes up about 60 from 0.1% to 10% of its weight of polyalkylene imine. In general the larger the proportion of imine taken up by the fiber, the greater will be the shrinkage protection afforded. It is also obvious that the degree of shrinkproofing attained will vary depending on such factors as the original characteristics of the fiber, the type of polyalkylene imine chosen and so forth. In any particular situation the fiber may be subjected to pilot ex-

periments, applying different proportions of the chosen polyalkylene imine and selecting the conditions which give the desired degree of shrinkproofing.

The process of this invention is particularly adapted for the treatment of wool but may also be applied to other proteinaceous fibers such as mohair, fibers from fleece-bearing animals other than sheep and goats, animal hair, silk, fibers made from proteins such as zein, casein, peanut protein, keratin, etc. The proteinaceous fiber may be in the form of actual fibers or may be in the form of threads, yarns, woven or knitted materials, garments, etc.

The invention is further demonstrated by the following example which is given only by way of illustration but not limitation.

#### EXAMPLE

An aqueous solution was prepared containing 5% of polyethylene imine (molecular weight about 20,000 to 30,000). The solution had a pH of 11.3.

Samples of woolen cloth were immersed in the solution and the cloth was run through padding rolls to assist in wetting it with the treatment solution. The cloth samples picked up about 120% of their weight of the solution.

The cloth samples were then placed in an oven where they were subjected to a temperature of 120° C. One lot of the samples was subjected to this heat for 30 minutes, another lot for 60 minutes.

The cured cloth samples were weighed to determine the uptake of polyethylene imine. The shrinkage characteristics of the cloth samples were determined by subjecting them to a laundering operation in which the cloth was violently agitated in a 0.5% solution of sodium oleate at 40° C. with a cloth to solution ratio of 1:50, the area of the cloth being measured before and after laundering. With this method of laundering, untreated cloth samples gave an area shrinkage of 36%.

Also, samples of the cloth which had been subjected to the above polyethylene imine treatment and curing were washed for 2 hours in running hot (55° C.) water. After this washing treatment the samples were dried and the residual polyethylene imine content was determined as well as shrinkage by the above laundering treatment.

The results obtained are set forth in the following table:

*Properties of woolen cloth impregnated with 5% solution of polyethyleneimine and cured at 120° C.*

| Sample.....                          | A  | B  |
|--------------------------------------|----|----|
| Curing time at 120° C., minutes..... | 30 | 60 |

#### PROPERTIES BEFORE HOT WATER EXTRACTION

|                                           |      |      |
|-------------------------------------------|------|------|
| Uptake of polyethyleneimine, Percent..... | 3.62 | 4.25 |
| Area Shrinkage, Percent.....              | zero | zero |

5

#### PROPERTIES AFTER WATER EXTRACTION

|                                           |      |      |
|-------------------------------------------|------|------|
| Uptake of polyethyleneimine, Percent..... | 3.49 | 2.25 |
| Area Shrinkage, Percent.....              | 1.88 | zero |

10

The following experiment demonstrates the adverse effect of acid conditions in the treating bath. A sample of woolen cloth was soaked in a 5% aqueous solution of polyethylene imine containing sufficient hydrochloric acid to give a pH of 5.0. The treated cloth was cured at 120° C. for 60 minutes then washed in hot running water (55° C.) for 2 hours. It was found that the uptake of polyethylene imine was 0.95% and the area shrinkage after laundering was 19.9%.

Having thus described the invention, what is claimed is:

1. A process for shrinkproofing protein fibers which comprises impregnating the protein fiber with an aqueous alkaline solution, having a pH about from 9 to 11, containing a preformed polyethylene imine having a molecular weight of about from 20,000 to 30,000, and curing the impregnated protein fiber at a temperature from about 75° C. to about 150° C.
2. A process for shrinkproofing wool which comprises impregnating wool with an aqueous alkaline solution, having a pH about from 9 to 11, containing a preformed polyethylene imine having a molecular weight of about from 20,000 to 30,000, and curing the impregnated wool at a temperature from about 75° C. to about 150° C.
3. The process of claim 2 wherein the solution of preformed polyethylene imine has a pH of about 11.
4. The process of claim 2 wherein the impregnated wool is cured at about 120° C. for about one hour.

#### References Cited in the file of this patent

#### UNITED STATES PATENTS

|           |                     |                |
|-----------|---------------------|----------------|
| 2,131,145 | Schlack .....       | Sept. 27, 1938 |
| 2,202,169 | Schlack .....       | May 28, 1940   |
| 2,269,997 | Berchet .....       | Jan. 13, 1942  |
| 2,526,637 | Cupery .....        | Oct. 24, 1950  |
| 2,553,696 | Wilson .....        | May 22, 1951   |
| 2,677,681 | Gill .....          | May 4, 1954    |
| 2,696,448 | Hammer et al. ..... | Dec. 7, 1954   |
| 2,817,602 | Pardo .....         | Dec. 24, 1957  |